

# UNITED STATES PATENT OFFICE.



## ALLOY-COATING PROCESS.

1,144,524.

Specification of Letters Patent. Patented June 29, 1915.

No Drawing.

Application filed January 9, 1913. Serial No. 740,922.

*To all whom it may concern:*

Be it known that I, JAY C. BENEKER, a citizen of the United States, residing at Cincinnati, in the county of Hamilton and State of Ohio, have invented certain new and useful Improvements in Alloy-Coating Processes, of which the following is a specification.

This invention proposes a method where-  
10 by a uniform and continuous alloy film of a hard, durable, physical character and of a non-corrosive and comparatively inactive chemical nature may be readily yet tenaciously applied to exposed surfaces of sheet iron, and more specifically this invention deals with the successful production as an article of manufacture of a film of hard antimony lead intimately amalgamated with commercial iron.

20 It is well known that ordinary commercial sheet iron is readily corrodible when exposed to outdoor atmospheric conditions and for many years various expedients have been resorted to to protect such surfaces. Thus, during the process of finishing such sheets preparatory to their use for building purposes, they have been commonly coated with metallic tin, or when a cheaper product was desired, with metallic zinc. By

30 reason of the cost of tin plate, on the one hand, and certain unsatisfactory features of zinc plate, on the other hand, many futile attempts have heretofore been made to coat iron successfully with other available metals.

I have discovered a process whereby soft lead may be applied to iron in a way satisfying all commercial requirements and the product is well adapted to resist corrosion and will meet all ordinary conditions, but by reason of the very soft ductile character of lead, such product is not as wear-resisting as would be desirable for some purposes. In seeking to attain a harder surface of film, I have found that lead alloyed with from three to thirteen per cent. of

ried out by preparing a melted bath of lead containing a suitable proportion of antimony, say about five per cent., and main-  
taining in said bath a small percentage 50 of my amalgamating metal exemplified by cadmium, say from two tenths per cent. to one per cent. This bath should preferably be maintained at as low a temperature as will be consistent with complete fusion and 65 the iron sheets may be passed continuously through such bath. At the point of entry, it is desirable to cover the bath by a layer of molten zinc chlorid to which a little hydrochloric acid may be added so as to 70 form a suitable flux for the purpose of keeping clean the bath and also chemically cleaning the iron surface and bringing it into a condition such that it will through the fur-  
ther agency of the cadmium be perfectly 75 amalgamated with the antimony lead bath when it is submerged therein. At the exit end of the bath, it is also preferable to maintain an overlying layer of palm oil preferably also submerging and keeping 80 clean the rollers or other means for squeez-  
ing off or otherwise ridding the outcoming plate of unnecessary amounts of the anti-  
mony lead.

While exceedingly simple this process is 85 most effective in attaining perfect results. By increasing the amount of antimony up to the eutetic proportion *i. e.* thirteen per cent. antimony, the melting point is re-  
duced to about two hundred and thirty de- 90 grees C. or about that of tin, and this makes the use of palm oil as a supernatant exit flux particularly feasible inasmuch as its 95 tendency to take fire is reduced to a very slight point. By adding varying amounts of antimony to a lead bath containing what I term an amalgamating element, *i. e.* a metal more positive than iron and yet freely miscible with lead, such as cadmium, a coating is obtainable quite free from pin holes 100 and at the same time hard and durable. It is very resistant to atmospheric conditions and neither rain water nor sulfuric acid

